

Nov. 30, 1943.

A. P. SHEPARD

2,335,316

APPARATUS FOR CONDITIONING METAL SURFACES FOR SPRAY METAL BONDING

Filed Nov. 25, 1940

2 Sheets-Sheet 1

FIG.1.



FIG.2.



FIG.3.



FIG.4.



INVENTOR.

ARTHUR P. SHEPARD,  
Louis Burges  
ATTORNEY,

BY

Nov. 30, 1943.

A. P. SHEPARD

2,335,316

APPARATUS FOR CONDITIONING METAL SURFACES FOR SPRAY METAL BONDING

Filed Nov. 25, 1940

2 Sheets-Sheet 2

FIG.5.



FIG.6.



FIG.7.



FIG.8.



INVENTOR.

ARTHUR P. SHEPARD.

Louis Berger,  
ATTORNEY.

BY

## UNITED STATES PATENT OFFICE

2,335,316

## APPARATUS FOR CONDITIONING METAL SURFACES FOR SPRAY METAL BONDING

Arthur P. Shepard, Forest Hills, Long Island, N. Y., assignor to Metallizing Engineering Company, Inc., Long Island City, N. Y., a corporation of New Jersey

Application November 25, 1940, Serial No. 366,957

2 Claims. (Cl. 80—5.1)

This is a continuation in part of my application Serial No. 221,650, filed July 27, 1938.

The invention relates to a new and useful apparatus for conditioning metal surfaces for spray metal bonding, and will be understood from the following description read in conjunction with the drawings in which—

Fig. 1 is an enlarged cross-section through a metal block having a pitted surface;

Fig. 2 is an enlarged section through a metal block having a grit blasted surface;

Fig. 3 is a cross-section through one embodiment of the invention;

Fig. 4 is a side view of part of the construction shown in Fig. 3;

Fig. 5 is an enlarged edge view of part of the construction shown in Fig. 4;

Fig. 6 illustrates an enlarged cross-section through a metal block having a surface prepared with a tool having teeth of an apex angle in excess of 120°;

Fig. 7 is an enlarged cross-section through a metal block showing a surface prepared with a tool having large and widely spaced teeth;

Fig. 8 is an enlarged cross-section through a metal block showing a surface obtained by the application of the tool in accordance with the invention.

The application of metal coatings to metal surfaces by metal spraying is achieved by the use of a metal spray gun, i. e., a device by which metal is fed to a heating zone from which zone metal particles, at least some of which are molten or in a heat plastic condition, are propelled against the object or surface by a blast of air or other gas. In order to obtain a coating on the object or surface sprayed, it is essential that the metal particles as they impinge upon the surface sprayed enter into a satisfactory bond with such surface. If the bond is too low, no spray metal coating is formed as the spray metal will not adhere to the surface and is either blown off by the force of the blast from the spray gun, or, it forms flakes upon the surface sprayed, these flakes curl, thus preventing the formation of the desired coating, alternatively, even if a coating is formed, the same will warp, peel, or loosen when worked upon if the spray metal bond to the base is not sufficiently high to prevent this.

For the purpose of obtaining a proper bond between spray metal and a metal base, it is requisite that the surface to be sprayed have a certain type and degree of roughness, principally characterized by two requirements. The first is that the surface not only be very rough, but that it

have a particular kind of roughness, i. e., a roughness in which the depressions are overhung by projections of metal so as to provide undercut cavities. These cavities act as minute dove-tailed keyways and interlock with the sprayed metal particles to form a strong bond. If the overhanging metal projections and dove-tailed cavities are absent, the bond between the spray metal and the base will not be satisfactory, no matter how rough or pitted a surface may otherwise be as, for example, a surface of the type obtained by knurling or the like, illustrated by numeral 50 in Fig. 1.

The second essential requirement for the surface roughness is that the indentations and metal projections be of a particular size and spacing. Since the size of the sprayed metal particles is very fine, the depressions and projections of the roughened surface must also be sufficiently fine to form a proper interlocking structure. On the other hand, the roughness represented by the depressions and projections must not be too fine, as otherwise the metal particles could not penetrate into the depressions and hence no satisfactory bond could be secured.

A surface of the desired type roughness meeting both of the primary requirements for satisfactory spray metal bonding, is conventionally obtained by sand or grit blasting, using as the recommended material a #30 to #40 sharp, angular steel grit which, when blown through a proper nozzle with an air pressure of approximately 90 to 100 pounds per square inch, will produce a very rough and irregular surface on the metal base being blasted, having a multiple number of closely spaced dove-tailed cavities. Such sand or grit blasted surface is, for instance, illustrated by numeral 51 in Fig. 2 which shows an enlarged section through a metal block, the surface of which was grit blasted in this manner.

The tool in accordance with my invention is designed to simulate as closely as possible the type of roughened surface which is produced by grit or sand blasting and which meets the essential requirements for satisfactory spray metal bonding to a metal base. The tool thus eliminates the costly operation of blasting; it replaces the expensive grit blasting equipment and permits the roughening operation, if desired, in the same machine tool in which machining and spraying is to be carried out, thereby obviating one or more extra machine set-ups.

The instrument which I have invented and which may be utilized to treat a metal surface in simulation of sand or grit blasting so as to strong-

ly bond thereto applied spray metal may be conveniently described in connection with the preferred embodiment of my invention illustrated in Figs. 3, 4 and 5. As there shown, a group 1 of steel discs is carried by spool 2 and held by nut 3 and lock-nut 4 in contact with the spool and with one another. Spool 2 and disc assembly 1 are carried by shaft 5. Spool 2 is secured between shoulder 6 integral with shaft 5 and machine screw 7. By removing screw 7, spool 2 and disc assembly 1 may be removed from the shaft when desired and replaced by a new spool and disc assembly. Shaft 5 is rotatably carried in ball-bearings 10 and 11 mounted in block 12 provided with extension 13. This extension is of such size and proportions that it may be inserted and secured in the ordinary lathe tool post or similarly mounted in the tool holder of a machine tool such as a planer, shaper or boring mill. In an alternative embodiment of this phase of my invention, spool 2 and disc assembly 1 may be similarly carried on a shaft projecting beyond the spool on either side and each end of this shaft may be mounted in a bearing, which bearing is carried by one tyne of a two-tyned fork forming a tool which may similarly be manipulated by hand or secured in a machine tool post. The construction shown in Fig. 3 has, however, the advantage that if used on work which has a projecting shoulder the disc assembly may be worked closer to the shoulder than the alternative type in which the disc assembly is carried between the tynes of a forked handle.

Each of the discs 8 (Fig. 4) is provided with teeth 9. The teeth of the assembled discs are not in alignment but are staggered with respect to one another. This is illustrated in Fig. 5 in which 15 designates the vertices of the teeth and 16 the valleys between the teeth of alternate discs, while 17 designates the vertices and 18 the valleys between the teeth of the other discs.

The arrangement of the plurality of rows of sharp teeth, in such manner that some of the teeth of some rows are out of line with some of the teeth of other rows is essential for otherwise the teeth will tend to continue to relocate in the depressions first made and form a surface of the type illustrated in connection with Fig. 1 having no dove-tailed cavities and being not a satisfactory spray metal bonding surface.

The apex angle of the teeth is critical for the successful operation of the device as I have found it necessary for the purpose of obtaining the proper type of surface roughness to get a reasonably narrow hole and then by a further action of the tool to split or peen the projection adjacent the hole so that the same will overhang the hole. When the apex angle of the teeth is too great, i. e., in excess of approximately 120°, such result cannot be achieved to a satisfactory degree for the hole produced by such teeth is too wide in relation to its depth to permit the edges to become properly peened over the hole by the subsequent action of the tool. This is for instance illustrated in Fig. 6 which represents a type of surface (52) produced by a tool with an apex angle greater than 120° and which shows the surface, though cut and roughened, yet to have insufficient overhanging projections to secure the proper bond between the spray metal and the metal base. On the other hand, if the apex angle of the teeth is less than approximately 45° the teeth will break and become dull under the severe action to which they are subjected which is true even if the teeth are made of hardened

tool steel. In most cases, however, I prefer, for best results, an apex angle of the teeth of approximately 90°.

The size and spacing of the teeth on each of the rows of teeth of the tool in accordance with the invention is also critical for the production of a satisfactory spray metal bonding surface. I have discovered it essential to provide for a pitch of rows of teeth of not in excess of approximately  $\frac{3}{4}$ " and a pitch of the teeth in the direction of the circumference of each row of teeth not less than approximately 30 nor more than approximately 4 teeth per linear inch. If the teeth do not meet these dimensional and spacing requirements and are for instance too large and spaced too far apart, and are consequently forced too deeply into the base to which the tool is applied, an unsatisfactory type of surface results, which surface is, for instance, typified by the solid surface lines 53 in Fig. 7. If the metal of the base to be treated by the tool would possess an unlimited amount of ductility, a surface such as is shown by the combination of the solid and dotted surface lines (Fig. 7) would be produced. Such a surface, however, cannot result because of the limits of ductility of the base metal, as the projections (54) will break off when drawn or worked through too great a distance by the repeated action of the tool, leaving the surface as indicated by the solid surface line without any appreciable amount of satisfactory overhanging projections essential to the anchoring of the spray metal when applied to such surface. Furthermore, a tool having teeth that are too large and too widely spaced would be substantially incapable of producing such close spacing of the individual cavities essential for the conditioning of a metal surface for spray metal bonding as is represented by the relatively fine texture of a sand or grit blasted surface.

I have found it necessary to so construct the tool that the individual teeth will strike the metal with as near as possible perpendicular motion to the surface being prepared. This gives a chopping and peening effect which first cuts holes and then flays and peens the projections so that some of the metal of the projections overhangs the hole. The proper relative tooth motion to the surface to be worked results when the discs carrying the rows of teeth are freely rotatable on their axis while the rows of teeth in the tool assembly are rolled over the work piece. If there is any undue amount of frictional drag in the rotation of the discs, the teeth will drag across the surface to be prepared and even a slight amount of such drag will result in a surface of unsatisfactory spray metal bonding characteristics. This is due to the fact that if there is any relative motion tangential to the surface being prepared, the teeth will cut out a smooth hole and after the first series of holes is produced, subsequent action of the teeth when having any frictional drag, will cut off the very delicate projections of metal rather than splitting and peening them as is required.

In the practical application of the tool in accordance with my invention, the base to be sprayed is worked with the tool by moving the same back and forth over the surface until the desired roughness is obtained. The thus roughened surface does not present a succession of holes corresponding to the form of the disc teeth since the teeth do not track or mesh in the surface of the work but on the contrary, come down at random and in such a way, as above-pointed

out, that the surface between the teeth marks first formed is splayed and peened by subsequent impacts with the teeth to form minute cavities with overhanging outer edges. The base to be sprayed upon is preferably secured in an appropriate metal working machine, as, for instance, a lathe or planer while the tool is preferably secured in the tool holder of the machine and acts upon the surface of the base to be treated passing over and in contact with the same. The surface obtained on a metal base by the application of the tool in accordance with the invention is, for instance, illustrated in Fig. 8. The surface (54) there shown closely resembles that of a sand or grit blasted surface.

The foregoing description is furnished by way of illustration and not of limitation and it is, therefore, my intention that the invention be limited only by the appended claims or their equivalents wherein I have attempted to claim broadly all inherent novelty.

I claim:

1. A tool for producing a simulated sand blasted surface on metal for spray metal bonding, comprising a piece adapted to be held in a machine tool holder, a shaft mounted in said piece and a wheel carried by said shaft comprising a plurality of circumferential rows of metal peening and splaying teeth, at least the majority of said teeth each defining an apex angle of not in excess of approximately  $120^\circ$  and not less than approximately  $45^\circ$ , said wheel being freely rotatable

about the axis of said shaft, the peening and splaying surfaces of the teeth of at least some of said rows being out of line with respect to the peening and splaying surfaces of the teeth of other rows, at least the majority of adjacent rows of teeth having a side spacing substantially parallel to said axis of not in excess of approximately  $\frac{1}{4}$ " and the teeth of at least the majority of said rows of teeth having a circumferential pitch of not less than approximately 30 nor more than approximately 4 teeth per linear inch.

2. A tool for producing a simulated sand blasted surface on metal for spray metal bonding comprising a piece adapted to be held in a machine tool holder, a shaft mounted in said piece and a plurality of toothed metal discs carried by said shaft and freely rotatable about the axis of said shaft, at least the majority of said teeth being metal splaying and peening teeth and each defining an apex angle of approximately  $90^\circ$ , the peening and splaying surfaces of the teeth of at least some of said discs being out of line with respect to the peening and splaying surfaces of the teeth of other discs, at least the majority of adjacent toothed discs having a side spacing substantially parallel to said axis of not in excess of approximately  $\frac{1}{4}$ " and the teeth of at least the majority of said toothed discs having a circumferential pitch of approximately 18 teeth per linear inch.

ARTHUR P. SHEPARD.